

## UNITED STATES PATENT OFFICE

2,389,652

METHOD OF EXTINGUISHING FIRES AND  
FLUID USED THEREIN

Lewis G. Morris Timpson, Plainfield, N. J.

No Drawing. Application July 23, 1943,  
Serial No. 495,952

6 Claims. (Cl. 252—8)

The present invention aims to provide an improved method of extinguishing fires.

Another object is to provide a fire-extinguishing fluid which will have both relatively high and relatively low boiling point constituents in suitably balanced proportions adapted to blanket and extinguish flames.

Another object is to provide fire-fighting equipment of light weight and great effectiveness.

The invention has been developed more particularly in working out a method of smothering and extinguishing forced-draft fires of the type exemplified by aircraft fires, and in compounding a composition for use in fire-fighting apparatus designed for extinguishing such fires. For the purpose of disclosure of the principles of the invention such an embodiment will be more particularly described, but it will be understood that the principles may be variously embodied as the requirements of particular uses demand.

Fire-fighting equipment and extinguishing agents for aircraft fires are subject to certain obvious special requirements. The agent and its container should be of as light weight as possible. Liquid compositions used should not freeze at the low temperatures to be met with and should not have too high a vapor pressure at the highest temperature of storage or of use. If the fire-extinguishing liquid is to be shipped by ordinary freight the vapor pressure should be less than 25 pounds per square inch, gauge pressure, at 70 degrees F., to comply with I. C. C. Freight Tariff Rule 4. The disagreeable and toxic effects should not be intolerable nor dangerous. The extinguishing agent is more effective if it acts quickly and if it smothers the fire.

The nature and objects of the invention will be better understood from a description of a particular illustrative embodiment thereof. The method involves applying to the fire a gas or vapor in such manner that in part the fire will be smothered and in part the flame will be carried away and will not flash back to the combustible material. The invention provides an improved composition compounded to form an effective combination of gases or vapors when suitably applied to a fire.

Compositions which have proved particularly effective in extensive tests under rigid conditions are:

|                            | Example A | Example B | Example C |
|----------------------------|-----------|-----------|-----------|
|                            | Percent   | Percent   | Percent   |
| Methylbromide.....         | 5         | 5         | 5         |
| Ethylbromide.....          | 90        | 85        | 80        |
| Ethylenechlorobromide..... | 5         | 10        | 15        |

These compositions will not freeze at 100 degrees below zero C. The proportions of the sev-

eral ingredients, respectively, may vary considerably and diluting ingredients, or other active ingredients, may be added. Preferably the ethylbromide forms a major proportion of the effective ingredients and methylbromide and ethylenechlorobromide constitute minor proportions.

Good fire-extinguishing action can be obtained if the principal active ingredients are present in the following preferred proportions relative to one another:

|                             | Per cent |
|-----------------------------|----------|
| Ethylbromide .....          | 70 to 90 |
| Methylbromide .....         | 5 to 10  |
| Ethylenechlorobromide ..... | 5 to 20  |

The foregoing proportions mentioned as preferred are not to be construed as defining sharp limits but it has been found that there are definite advantages to be obtained if the ethylbromide constitutes a preponderance, and preferably two-thirds or more of the three-part compound. As much as about 5% of methylbromide is preferred, although half such amount is quite effective. An excess of 15% is not necessary in the composition and may increase the toxicity beyond reasonably permissible limits.

Each ingredient of the composition serves its particular purpose. Methylbromide is a particularly effective fire extinguisher. It is normally a heavy gas at temperatures above 4.5 degrees C. and effectively blankets and extinguishes oil and gasoline fires. This gas, however, is highly toxic. By dilution, as with the ethylbromide present, its toxicity is reduced to within tolerable limits. Although the methylbromide present constitutes a minor proportion it is of major importance as an effective fire-extinguishing ingredient.

Ethylbromide has been discovered to possess good fire-extinguishing properties, especially in the composition described, although it is otherwise described in the literature. Boiling at 38 degrees C., it is a relatively heavy gas and particularly effective for extinguishing forced-draft oil and gas fires. The combination of low boiling point and high boiling point elements is considered to be decidedly better than either alone.

Ethylene chlorobromide is used in a relatively minor proportion. Having a boiling point of about 106 degrees, it brings down the vapor pressure of the mixture as a whole. Preferably the proportion present in the composition is sufficient to insure a vapor pressure of less than 25 pounds gauge at 70 degrees F. and therefore within the limits of I. C. C. Freight Tariff Rule 4. Low vapor pressure permits use of a less strong and lighter-weight container.

When increasing the methylbromide content in order to improve the fire-extinguishing effectiveness, though at the expense of greater toxicity, the vapor pressure may be kept down by in-

easing also the proportion of ethylenechlorobromide. It is desirable especially for airplane fires that a sufficient volume of the low boiling point extinguishing gas be provided.

The preferred method of using compositions having as principal effective ingredients the chemical compounds mentioned, or their equivalents, respectively, involves applying fire-extinguishing liquid directly upon the burning mass. The fire-smothering gas or vapor will be released by the heat of the fire to extinguish the flame. If the liquid be applied as a fine spray the forced draft evaporation is quicker and the action extremely effective. The exact manner of the action of vapors to extinguish fire is not completely known but in some instances, at least, the vapors evolving from the liquid projected on to the fire seem to envelop the mass of burning gas and carry it away without permitting the flame to flash back to the combustible material.

In carefully conducted tests it has been established that the mixture of vapors produced from the compositions described are particularly effective for extinguishing fires of the type occurring in airplane power plants. At the same time the toxicity of the gaseous mixture is not beyond permissible limits for the crew to endure.

The foregoing particular description is illustrative of the principles involved but is not intended as defining the limits of the invention. Various modifications and various other embodiments may be developed without departing from the spirit of the invention as defined in the appended claims.

What is claimed is:

1. The method of extinguishing fires which comprises applying to the fire a liquid including as its principal effective ingredients methyl-

bromide, ethylbromide and ethylenechlorobromide in proportions approximating 4 to 10%, 75 to 85% and 10 to 20%, respectively, to produce fire-extinguishing vapors.

2. A vapor-forming fire-extinguishing liquid comprising as its principal effective ingredients about 70 to 90% ethylbromide, 5 to 10% methylbromide, and 5 to 20% ethylenechlorobromide.

3. A vapor-forming fire-extinguishing liquid comprising as its principal effective ingredients minor proportions of methylbromide and ethylenechlorobromide and a major proportion of ethylbromide whereof the vapor pressure at 70 degrees F. is less than 25 pounds above atmospheric pressure.

4. The method of extinguishing fires which comprises applying to the fire a liquid containing 2½% or more methylbromide, a preponderance of ethylbromide and sufficient ethylene chloro bromide to reduce the vapor pressure of the composition at 70 degrees F. to about 25 pounds per square inch above atmospheric pressure.

5. The method of extinguishing a forced draft fire which comprises applying to the fire in the forced draft a fine spray of a liquid including as principal effective ingredients about 2½% or more methylbromide, about 4 to 10% ethylene chloro bromide and a major proportion of ethylbromide.

6. A vapor forming, fire-extinguishing liquid comprising as principal effective ingredients 2½ to 15% methylbromide, a major proportion ethylbromide and sufficient ethylene chloro bromide to reduce the vapor pressure at 70 degrees F. to less than 25 pounds per square inch above atmospheric pressure.

LEWIS G. MORRIS TIMPSON.